

# UNITED STATES PATENT OFFICE.

ALBERT L. MARSH, OF DETROIT, MICHIGAN, ASSIGNOR TO HOSKINS MANUFACTURING COMPANY, OF DETROIT, MICHIGAN, A CORPORATION OF MICHIGAN.

## THERMO-ELECTRIC ELEMENT.

1,076,438.

Specification of Letters Patent.

Patented Oct. 21, 1913.

No Drawing.

Application filed September 30, 1912. Serial No. 723,197.

To all whom it may concern:

Be it known that I, ALBERT L. MARSH, a citizen of the United States, residing at Detroit, in the county of Wayne and State of Michigan, have invented a new and useful Thermo-Electric Element, of which the following is a specification.

My invention relates to a novel thermo-electric element.

10 Pure nickel has long been used as a positive element in thermo electric couples, and it is known to give a good millivoltage when associated with any of the known negative elements. However, nickel is of a peculiar 15 unreliable nature. The causes for this fault of nickel are obscure in their nature and not fully understood, but in practice it is found that while occasionally a pure nickel element will have a normal life, almost always 20 it develops extremely brittle spots so that it breaks under the ordinary handling to which it is necessarily subjected in practice. Particularly, when used in fuel furnaces, does this difficulty appear, and I am therefore inclined to believe that the cause of the 25 increase of brittleness is the presence of reducing gases which seem to enter into some sort of a chemical union, possibly of a very unstable nature with the nickel. It is known 30 that nickel unites at certain temperatures with carbon monoxide, and a reaction of this character may have something to do with the well-known treachery of nickel for the purpose intended.

35 I have discovered that the addition of silicon to the nickel to a large extent eliminates this difficulty of nickel without effecting or materially changing its millivoltage when used as a thermo-electric element. I prefer to add the silicon in from 3 to 5%, and with my present knowledge of the art of rolling and drawing metals I have not succeeded in satisfactorily working any element in which the silicon runs above 7%, 45 although I do not intend to state that that is the highest limit to which it can be added and still form a workable alloy, for the reason that the art of working metals is constantly advancing and from time to time 50 metals are rolled, which were considered absolutely unworkable in the past.

To get the best result, I find it desirable to add in addition to the silicon a quantity of manganese, aluminum, or some other well-known deoxidizer, slightly in excess of the

amount required for deoxidizing purposes. This slight excess serves merely to render the metal more easily workable and there are doubtless other metals than deoxidizers which will have this same effect. In other 60 words, the nickel-silicon alloy seems to be slightly cold short, and the addition of a slight amount of manganese or aluminum, and probably many other metals, removes this shortness.

65 I have heretofore patented a positive thermo-electric element consisting of nickel and aluminum. The nickel-aluminum alloy is considerably better than the nickel, but the treacherous and unreliable character of the 70 nickel is more thoroughly removed by the addition of silicon than by the addition of aluminum. On the other hand, in the present state of my knowledge, I am of the opinion that the silicon-nickel cannot be 75 run at as high temperature as can the nickel-aluminum and, therefore, I prefer to use the present element for temperatures up to 2000° F., or thereabout, and the nickel-aluminum element for a higher temperature. 80 These statements, however, of comparative values are not intended to be absolute in their nature for the reason that they are based only on my present experience, and in practice, I find that variations in the purity 85 of the metal, the manner of working them and the like, bring out from time to time new properties or capacities. As a positive statement I can go no further than to say that the present element is very satisfactory 90 in temperatures up to 2000° F., that it is very much better than pure nickel, and that in practice at such temperatures at the present time I am using it in preference to the nickel-aluminum.

95 While I have described the preferred composition of my element, I do not intend to be limited to elements composed solely of the metals specified for the reason that it will be obvious to those skilled in the art, 10 that other metals may be added to the nickel-silicon without very material change, although doubtless some metals can be added which seriously upset its thermo electric properties. It is undoubtedly true, however, 10 that either iron or cobalt can be used in considerable percentages, as additions to the nickel-silicon alloy described without being seriously detrimental, although I have found in practice that cobalt changes the electro- 11

motive force temperature curve of a couple in which it is employed, so as to make the couple less desirable for electrical measurement purposes. Doubtless, other materials 5 can be added in the same way, without departing from the spirit of my invention.

What I claim as new and desire to secure by Letters Patent is:

1. A positive thermo-electric element consisting of nickel and silicon.
2. A positive thermo-electric element consisting of nickel and silicon, the silicon in proportion of from 3 to 5%.
3. A positive thermo-electric element consisting of nickel and silicon, with an added

quantity of an auxiliary adapted to remove shortness.

4. A positive thermo-electric element consisting of an alloy of nickel and silicon, with an added quantity of manganese as an auxiliary to remove shortness. 20

5. A positive thermo-electric element consisting of nickel and silicon, the silicon in the proportion of from 3 to 5%, with an added quantity of manganese to remove 25 shortness.

ALBERT L. MARSH.

In presence of—

J. G. ANDERSON,  
J. LANDESMAN.